

## UNITED STATES PATENT OFFICE

MEYRL M. FROST, OF CAPAC, MICHIGAN

## PRODUCTION OF FIBER ARTICLES

No Drawing. Application filed August 20, 1927, Serial No. 214,438. Renewed May 1, 1929.

The present invention relates to the production of articles of compressed fibrous materials and particularly of a process of producing such articles and the articles produced thereby.

Among the objects of the invention is an article of manufacture which is extremely compact, tough, waterproof and capable of taking an excellent finish.

Other objects will readily appear to those skilled in the art upon reference to the following description.

Heretofore, such articles of manufacture as chair or toilet seats, doors, boxes and the like have been usually made of wood pieces glued or otherwise secured together. Wood has been considered the only suitable material because of its plentifullness and also because of its low heat conductivity. However, due to its property of absorbing moisture, it is difficult if not impossible to build up an article, such as a toilet seat, from pieces of wood glued together and have the pieces adhere permanently.

The present process produces an article that is not built up of pieces but is of homogeneous composition, waterproof and has all of the advantageous properties of wood.

The process is carried out by first forming a fluent pulp of fibrous material, such as ground wood pulp or pulp of rag fiber, waste-paper, hemp, jute or even asbestos. To this pulp having preferably from four to twenty per cent solids is added rosin soap up to fifty per cent of the total solids. This mixture is agitated thoroughly and pumped into suitable dies where the water is expressed therefrom and the article formed under a pressure depending on the article to be produced up to six hundred pounds per square inch. The formed article is then removed from the die and dried and rough finished if necessary.

After the drying steps the article is then dipped in a solution of preferably sixty per cent pine oil and forty percent banana oil and allowed to remain a short time, say from three to ten minutes or longer if necessary to allow the said solution which is quite fluid to impregnate to some extent, after which

it is allowed to cool. If it is desired to completely impregnate, the article should remain in the said treatment for a considerable period. The thus treated article is then painted if desired and is ready to be marketed.

The treatment with the pine oil and banana oil by dipping and submerging for a short time is sufficient for ordinary purposes but, if desired to impregnate deeply pressure methods such as are used to impregnate other porous materials may be used. Such methods consist in submerging the article in the impregnating liquid in a closed vessel and subjecting the liquid to high pressure or in first exhausting and then subjecting to pressure.

This pine oil and banana oil impregnation and superficial coating renders the compressed fiber article waterproof and there is thus produced one that is strong and substantially permanent.

Now having described the invention and the preferred form of embodiment thereof it is to be understood that the said invention is to be limited not to the specific details herein set forth only by the scope of the claims which follow.

I claim:

1. The process of producing homogenous fiber articles which consists in forming a pulp of the fiber in finely divided conditions with water, mixing with said pulp rosin soap, expressing said water therefrom under high pressure drying and subjecting the molded article to an impregnation treatment with a solution of pine oil and banana oil.

2. The process of producing homogenous fiber article which consists in forming a pulp of the fiber in finely divided conditions with water, mixing with said pulp rosin soap expressing said water therefrom under a pressure of up to six hundred pounds per square inch, drying and subjecting the molded article to an impregnation treatment with a solution of pine oil and banana oil.

3. An article of manufacture comprising a hard tough body of finely divided organic fiber and rosin soap with a coating and at least a superficial impregnation with a solution of pine oil and banana oil.

MEYRL M. FROST. 100